

June 21, 1927.

F. J. BLACK

1,632,818

RING GEAR AND METHOD OF MAKING THE SAME

Filed June 27, 1922

Fig. 1.



Fig. 2.



Fig. 3.



Fig. 4.



Fig. 5.



Fig. 6.



Witnesses:

Edwin Trueb

Inventor:  
FRANK J. BLACK.

Anthony Usina  
his Attorney

Patented June 21, 1927.

1,632,818

# UNITED STATES PATENT OFFICE.

FRANK J. BLACK, OF CRAFTON, PENNSYLVANIA.

## RING GEAR AND METHOD OF MAKING THE SAME.

Application filed June 27, 1922. Serial No. 571,259.

This invention relates to gears and more particularly to ring gears and the method of manufacturing the same, and has for one of its objects the provision of a gear of this class that will be more durable, efficient, and less noisy in operation than gears heretofore made.

Another object is the provision of a gear of this class and method of making same having the novel features hereinafter described and illustrated in the accompanying drawings.

Heretofore ring gears have been formed from rolled steel slabs by forging the slabs into blanks substantially as shown in Figure 5 and then cutting teeth therein. The flow lines or grain of the metal of the rolled slabs necessarily extend or run lengthwise of the slab and, therefore, when a circular gear blank is formed from such slabs the flow lines or grain of the metal on two quarters of the blank run parallel with the cut of the teeth, thereby materially weakening the teeth in that area. Experience has shown that 99 per cent of the breaking out of the teeth on ring gears occurs in this area. Also ring gears formed from rolled steel slabs do not have uniform shrinkage when heat treated to harden them. Experience has shown that where the flow lines running parallel with the teeth in two quarters of the ring connect with the other two quarters, the shrinkage varies from .003 to .004 inches, thus producing a very noisy and often defective gear.

The present invention entirely overcomes these difficulties and provides a gear in which the flow lines or grain of the metal extends perpendicular with the cut of the teeth at all points on the gear.

Referring to the drawings, Figure 1 is an elevation of a rolled steel round used in carrying out the method of this application.

Figure 2 is a sectional elevation of the pierced blank formed from the round of Figure 1.

Figure 3 is a sectional elevation of the drawn tubular blank formed from the pierced blank of Figure 2.

Figure 4 is a sectional elevation of a ring gear blank cut from the tubular blank of Figure 3.

Figure 5 is a sectional elevation of the ring gear blank of Figure 4 after forging.

Figure 6 is a sectional elevation of the

ring gear blank of Figure 5 after the teeth have been cut thereon.

In carrying out this invention ingots are first rolled down to produce long rounds which are then sheared or otherwise cut to short lengths to form the blank rounds or cheeses 2 shown in Figure 1. The blank rounds 2 are then pierced lengthwise by any of the well known processes now in use to form the pierced blank 3 of Figure 2, having one closed head or end 4. The greater portion of impurities and poor metal are always found in the center of an ingot, and since the ingot is rolled to produce the round blanks 2, any impurities or poor metal will still be found in the center of the rounds 2, and when said rounds are pierced the piercing plug or tool will force the impurities and poor metal forward into the head or closed end 4 of the pierced blank 3, which head is cut from the blanks and scrapped, therefore eliminating this poor metal and impurities from the ring blanks.

The pierced blank 3 is further elongated, thinned, and worked by drawing it on a mandrel after the fashion of drawing seamless tubes or the like, to produce the tubular drawn blank 5 of Figure 3. The blank 5 is then cut into short lengths to form the ring blanks 6 of Figure 4, which are substantially the size of the finished gear.

The ring blanks 6 are then heated and forged to produce the forged ring blank 7 of Figure 5, which is the same shape and size as the finished gear. The blanks 7 are then milled or otherwise cut to form the teeth 8 on their one side face as shown in Figure 6.

It will be noted that all working of the metal in producing the blanks from the rolling of the ingot to form the rounds to the drawing operation used in producing the thin tubular blank 5 of Figure 3 is lengthwise of the longitudinal axis of the blanks and therefore the flow lines or grain of the metal necessarily extend or run parallel to the longitudinal axis and perpendicular to the cut of the teeth 8 around the entire gear.

After the blanks 7 have had the teeth 8 cut therein they are heat treated to harden them and finally ground to produce perfect finish required on such gears.

The primary novel feature of this invention lies in producing a ring gear in which the flow lines or grain of the metal runs

perpendicular to the cut of all the teeth, thus eliminating the weak area found in two quarters of the teeth on the ring gears heretofore produced, which teeth have necessarily had the flow lines or grain of the metal running parallel with the teeth.

I claim:—

1. In the manufacture of ring gears the steps comprising forming a tubular blank by piercing and drawing, cutting rings from said blank, and forming teeth on at least one side face of said rings.
2. In the manufacture of ring gears the steps comprising forming a tubular blank by piercing and drawing, cutting rings from said blank, and forging said ring to form, and cutting teeth on at least one side face thereof.
3. In the manufacture of ring gears the steps comprising forming a rolled steel round, piercing and drawing said round to

form a tubular blank, cutting rings from said blank, and forming teeth on at least one side face of said rings.

4. A ring gear formed from a drawn steel blank and in which the flow lines or grain of the metal runs substantially perpendicular to the cut of all the teeth.

5. In the manufacture of ring gears, the steps comprising forming a circular blank having the grain of the metal running in a line substantially parallel to the axis thereof, and forming teeth on at least one side face of said blank so that the grain of the metal will extend substantially perpendicular to the cut of the teeth.

6. A ring gear having the flow lines or grain of the metal running substantially perpendicular to the cut of all the teeth.

In testimony whereof I have hereunto set my hand.

FRANK J. BLACK.